# EUROPEAN PATENT APPLICATION

(11) **EP 1 967 617 A1**
(43) Date of publication of application: **10.09.2008**
(21) Application number: 07009995.7
(22) Date of filing: 18.05.2007
(51) Int. Cl.: D01D 5/00, D04H 3/00

(54) **Fibrous structures, processes and devices for preparing the same**

(30) Priority: 09.03.2007 GB 0704615
(71) Applicant: Universiteit Gent, 9000 Gent (BE)
(72) Inventor: Westbroek, Philippe, 9200 Dendermonde (BE); Van Camp, Tamara, 9000 Gent (BE); Braem, Jan, 8310 Sint-Kruis Brugge (BE); De Clerck, Karen, 9040 Sint-Amandsberg (BE)
(74) Representative: Bird, Ariane

(57) **Abstract**

An electrospinning device is described for producing nanofibrous porous structures. The device comprises two or more outlets (11) separated from one another by a distance of at least 1 cm and positioned in a first plane (12). The device also comprises a second surface (13) for receiving output from the outlets. A relative movement between the two or more outlets (11) and the second surface (13) can be applied in a first direction and second direction, the second direction being substantially perpendicular to the first direction. The second surface (13) thereby is facing the first plane wherein the outlets are positioned. The device furthermore comprises a voltage source (9) adapted to apply a potential difference between the first surface and the second surface. It furthermore may comprise a recipient for containing a solution or melt to be electrospun from the outlets and comprises a providing means for providing (10) the solution or melt to the outlets.

## Description

### Technical field of the invention

The present invention relates to a fibrous structure, a process and a device for manufacturing the same. In particular, the present invention relates to fibrous structures such as e.g. nanofibrous structures and their applications as absorption or filtration material such as in wound dressings, wipers, diapers, filtration, compound immobilization, inclusion of chemicals, etc.

### Background of the invention

Nanofibrous structures are useful in a variety of applications in the fields of clothing, filtering, medicine, cosmetics and defense. There is a strong interest in nanofibrous structures based on their high porosity for absorption, immobilization and inclusion of chemicals, solvent, solutions, melts and liquid phases. In many applications, such as wound burn treatment, teeth whitening gel immobilization, disinfecting solution immobilization, urine absorption and other applications where high absorption is preferred, an absorption capacity of about 5 mL.cm⁻² is preferably obtained. In the same applications large nanofibrous structures (e.g. for wound burn treatment a minimum dimension is 40 by 40 cm for a mat) are needed. In order to guarantee homogeneous absorption behaviour over the structure it is useful to obtain a regular thickness over the entire structure.

Nanofibrous structures can be produced using an electrospinning setup. A basic setup is shown in FIG. 1 and consists of a high voltage source 1, an anesthesia pump 2, the pump comprising a syringe 3 that contains a polymer solution 4 and the pump transporting polymer solution towards the tip of a metallic needle 5, said needle positioned in a spinneret 6, said spinneret comprising an upper 7 and a lower 8 conductive plate. An electrical field is applied over the upper and lower plate resulting in an extrusion ability of the polymer solution at the tip of the needle towards the surface of the lower element. The electrical field created, causes the polymer solution to overcome the cohesive forces that hold the polymer solution together. As a result of cohesive force compensation by the electrical field a jet will be drawn from the polymer solution droplet, which forms nano-dimensioned fibres, finally collected at the lower plate. Typical dimensions of the deposited structures are circular surfaces with a diameter of about 10 to 15 cm. Therefore, with a single nozzle system, it is not possible to obtain the large surface areas required for many applications in an economic feasible way.

Multi-nozzles apparatus have been described as attempts to enable upscaling of the electrospining process. Such a device is described in International patent application WO 2005/073442. In WO 2005/073442, a multinozzle electrospinning device is disclosed wherein a continuous nanofiber filament is formed by producing and twisting a nanofiber web. WO 2005/073442 does not disclose means to achieve the production of nanofibrous structures composed of straight fibers and/or non-crosslinked fibers and/or fibers of controlled diameter. Furthermore WO 2005/073442 does not disclose means to achieve the production of fibrous structures having a uniform thickness and/or a large width and/or a high strength.

There is therefore still a need in the art for a device and a method to produce fibrous (e.g. nanofibrous) structures with high porosity, large width, high mechanical strength and uniform thickness in an economic viable way. There is also a need for a device and a method to produce fibrous (e.g. nanofibrous) structures with enhanced filtration or liquid transportation properties.

### Summary of the invention

It is an object of the present invention to provide good devices or methods for producing fibrous (e.g. nanofibrous) structures. It is an advantage of embodiments according to the present invention that fibrous structures with high porosity are provided and methods for producing them. It is an advantage of embodiments according to the present invention that fibrous structures with large width and/or uniform thickness are provided and methods for producing them. It is also an advantage of embodiments according to the present invention that fibrous structures with improved mechanical strength are provided and methods for producing them. It is furthermore an advantage of embodiments according to the present invention that fibrous structures with good liquid uptake are provided and methods for producing them. It is also an advantage of embodiments according to the present invention that fibrous structures with good control release and filtration properties are provided and methods for producing them. It is an advantage of embodiments according to the present invention that fibrous structures can be provided in an economic viable way. It is an advantage of embodiments according to the present invention that fibrous structures with a combination of two or more of the above described advantages can be obtained.

The above objective is accomplished by a method and device according to the present invention.

The invention relates to an electrospinning device for producing fibrous structures, said electrospinning device comprising a set of two or more outlets for outputting solution or melt, said two or more outlets being arranged in a first plane, a second planar surface arranged parallel to said first plane, the second planar surface for receiving output from said two or more outlets, wherein said set of two or more outlets and said second planar surface are adapted to move relatively to each other, a voltage source for generating a potential difference between said set of two or more outlets and said second surface, providing means for providing said solution or melt to said outlets, characterized in that at least two neighbouring outlets of said two or more outlets are separated from one another by a distance of at least 1 cm. It is an advantage of embodiments according to the present invention that devices are provided allowing to produce fibrous structures with high porosity. At least two neighbouring outlets of said two or more outlets may be separated by a distance of at least 2 cm. It is particularly advantages to separate two neighbouring outlets by a distance of at least 4cm. Each two outlets of said at least two or more outlets may be separated from one another by a distance of at least 1 cm, advantageously a distance of at least 2 cm, more advantageously of at least 4 cm. In other words, there is at least one nozzle for which the distance to the closest other nozzle is at least 1 cm, advantageously at least 2cm, more advantageously at least 4cm. A majority or all of said two or more outlets may be separated from the other outlets by a distance of at least 1 cm, advantageously at least 2 cm, more advantageously at least 4 cm. It is an advantage of embodiments according to the present invention that devices are provided allowing production of fibrous structures that are strong, have high porosity and straight fibres.

The distance between said two or more outlets may be adapted for obtaining a fibrous structure comprising at least 50% of fibers substantially free of cross-links to neighboring fibers. It is an advantage of embodiments according to the present invention that devices are provided allowing production of fibrous structures wherein only a low degree of cross-linked fibers is present.

The distance between said two or more outlets may be adapted for obtaining a fibrous structure comprising at least 50% of straight fibers. The device may be adapted for applying a relative movement between said two or more outlets and said second surface in a first direction and in a second direction, different from said first direction. The second direction may be perpendicular to said first direction. The second direction may be parallel to said first plane. Alternatively, the second direction may be perpendicular to said first plane.

The two or more outlets may be adapted to be movable reciprocally in said first direction.

The device may comprise control means for varying the diameter of the produced fibres.

The means for varying the diameter of the produced fibres may be control means for altering the distance between said first plane and said second planar surface during the production of the fibrous structure.

The present invention also relates to an electrospinning device for producing a fibrous structure, said electrospinning device comprising one or more outlets for outputting solution or melt, said two or more outlets being arranged in a first plane, a second planar surface, for receiving output of said two or more outlets, the second planar surface arranged parallel to said first plane, a voltage source for generating a potential difference between said one or more outlets and said second planar surface, providing means for providing a solution or melt to said outlets, characterized in that said device comprises control means for varying the diameter of the produced fibres.

The means for varying the diameter of the produced fibres may be control means for altering the distance between said first plane and said second planar surface during the production of the fibrous structure.

The device may be adapted for generating a plurality of fibers, whereby at least 50% of said plurality of fibers may comprise an average diameter between 3 and 2000 nm. The device may be adapted for using a polymer solution or melt comprising at least one of a polyamide, polystyrene, polycaprolactone, polyacrylonitrile, polyethylene oxide, polylactic acid, polyacrylic acid, polyesteramide, polyvinyl alcohol, polyimide, polyurethane, polyvinylpyrrolidon, collagen, cellulose, chitosan, methacrylates, silk or metal.

The present invention also relates to a method for producing fibrous structures, said method comprising the steps of moving a set of two or more outlets, for outputting solution or melt, said set being comprised in a first plane, relatively to a second planar surface, for receiving output of said two or more outlets, applying a potential difference between said set of two or more outlets and said second planar surface, and, during said moving and applying, providing a solution or melt to said outlets, wherein said two or more outlets are separated from one another by a distance of at least 1 cm. At least two neighbouring outlets of said two or more outlets may be separated by a distance of at least 1 cm, advantageously at least 2cm, more advantageously at least 4cm. Each two of said at least two or more outlets may be separated from one another by a distance of at least 1 cm, advantageously at least 2cm, more advantageously at least 4cm.

The moving step may comprise adapting the distance between said set of two or more outlets and said second planar surface.

The present invention also relates to a method for producing fibrous structures, said method comprising the steps of adapting the distance between a set of one or more outlets for outputting solution or melt, said set being comprised in a first plane, and a second planar surface for receiving output of said two or more outlets, applying a potential difference between said set of one or more outlets and the second planar surface, and providing a solution or melt to said outlets.

The distance may be adapted by providing a relative movement between said set of outlets and said second planar surface in a first direction and a second direction perpendicular to said first direction and perpendicular to said first plane. The moving step may be performed such as to achieve a predefined distance between said set of outlets and said second planar surface, and, while performing the applying step and providing step, at least one of said set of outlets and/or said second planar surface may be moved reciprocally in a first direction and in a second direction perpendicular to the first direction and parallel to said first plane. The method furthermore may comprise iterating the first moving step and the reciprocally moving step for a predetermined number of times, wherein the sense of movement is reversed between each iteration.

The method may be adapted for generating a plurality of fibers, whereby at least 50% of said plurality of fibers comprises an average diameter between 3 and 2000 nm. The method may be adapted for using a polymer solution or melt comprising at least one of a polyamide, polystyrene, polycaprolactone, polyacrylonitrile, polyethylene oxide, polylactic acid, polyacrylic acid, polyesteramide, polyvinyl alcohol, polyimide, polyurethane, polyvinylpyrrolidon, collagen, cellulose, chitosan, methacrylates, silk or metal.

The present invention relates to an electrospun fibrous structure, the structure comprising at least 50% of straight fibers, wherein at least 50% of straight fibers consists of 50% or more fibres having segments substantially straight over a distance of 5 µm.

The electrospun fibrous structure may comprise at least 50% of fibers that is substantially cross-link free with respect to neighboring fibers.

The electrospun fibrous structure may at least 50% of randomly oriented fibers.

The electrospun fibrous structure may have a porosity of at least 65%.

50% or more of its fibers may have an average diameter between 3 and 2000 nm.

The present invention also relates to an electrospun fibrous structure comprising two or more layers, wherein each of said layers is composed of fibers having an average diameter different from the average diameter of the fibers of an adjacent layer.

The present invention furthermore relates to a filtrating or an absorbing device comprising an electrospun fibrous structure as described above.

The present invention also relates to a controller for controlling an electrospinning device, the controller being adapted for performing any of the above described methods.

In one aspect, the present invention relates to an electrospinning device for producing nanofibrous structures having a porosity of at least 65%, said electrospinning device comprising a first surface comprising three or more outlets, said first surface being adapted to be movable in a first direction, a second surface adapted to be movable in a second direction, e.g. at an angle to the first direction such as optionally substantially perpendicular to said first direction, said second surface facing said first surface, a voltage source adapted to apply a potential difference between said first surface and said second surface, a recipient for containing a solution or melt to be electrospun from said outlets, and means for providing said solution or melt to said outlets. As an optional feature, the three or more outlets can be separated from one another by a distance of at least 1 cm.

As an optional feature, said recipient may contain a polymer solution or melt.

As an optional feature of this first embodiment, the spinneret may allow the production of nanofibrous structures with a width between 15 and 10.000 cm.

As an optional feature, the non-woven nanofibrous structures comprise nanofibers having a diameter between 10 and 2000 nm, advantageously below 700 nm.

As another optional feature, the lower and the upper section are adapted to be moveable perpendicularly to each other.

As another optional feature, a voltage difference of between 100 V and 200000 V is applied over the upper and lower element of the spinneret.

As another optional feature, the spinneret further comprises a set of needles positioned at the upper plate, said needles releasing a polymer solution or a polymer melt flow, obtained through a pump.

As another optional feature, the needles are positioned in a triangle setup or a multiple thereof.

As another optional feature, the distance between the needles is between 1 and 100 cm.

As another optional feature, the pump rate of the polymer solution or melt per needle is between 0.01 and 500 mL h⁻¹.

As another optional feature, the polymer solution or melt used contains one of the following polymers or polymer classes: polyamides, polystyrenes, polycaprolactones, polyacrylonitriles, polyethylene oxides, polylactic acids, polyacrylic acids, polyesteramides, polyvinyl alcohols, polyimides, polyurethanes, polyvinylpyrrolidon, collagen, cellulose and related products, chitosan, methacrylates, silk and metal containing nanofibers.

As an optional feature, the solutions or melts may contain an additional compound, such as compounds with antibacterial, farmaceutical, hydrophobic/hydrophilic, anti corrosion, catalytic, oxidative/reductive and other properties.

As another optional feature, structures of nanofibers are obtained with a porosity between 65 and 99%

As another optional feature, structures of nanofibers are obtained, said fibers having a diameter between 3 and 800 nm.

As another optional feature, the device comprises a surrounding element over the spinneret to avoid instability and to allow solvent recuperation.

As another optional feature, the device comprises a temperature control system that allows to control the temperature in the range of 280 - 1500 K.

In a further aspect, the present invention relates to a method for producing nanofibrous structures having a porosity of at least 65%, said method comprising the steps of applying a potential difference between a first surface and a second surface, said first surface comprising three or more outlets, moving said first surface in a first direction while simultaneously moving said second surface in a second direction substantially perpendicular to said first direction, and providing a solution or melt to said outlets.

The three or more outlets are advantageously separated from one another by a distance of at least 1 cm.

In a third aspect, the present invention relates to nanofibrous polymeric structures having a porosity of at least 65% and a width comprised between 15 and 10000 cm.

In some embodiments, the present invention relates to a device to produce nanofibrous structures (see FIG. 2, FIG.3 and FIG. 4) from polymer solutions and polymer melts. The device comprises a high voltage source, a spinneret, said spinneret comprising a number of outlets such as e.g. needles, an upper, and a lower element (e.g. surface), means such as but not limited to a peristaltic pump or anesthesia pump for providing the solution or melt to the outlets, an optional surrounding element, and an optional temperature control system, said system may for instance comprise jacketed tubes and containers for liquid or oil based temperature control and gas heaters for environmental temperature control.

Particular and preferred aspects of the invention are set out in the accompanying independent and dependent claims. Features from the dependent claims may be combined with features of the independent claims and with features of other dependent claims as appropriate and not merely as explicitly set out in the claims.

Although there has been constant improvement, change and evolution of devices in this field, the present concepts are believed to represent substantial new and novel improvements, including departures from prior practices, resulting in the provision of more efficient, stable and reliable devices of this nature.

The teachings of the present invention permit the design of improved methods and apparatus for manufacturing fibrous structures with enhanced properties.

The above and other characteristics, features and advantages of the present invention will become apparent from the following detailed description, taken in conjunction with the accompanying drawings, which illustrate, by way of example, the principles of the invention. This description is given for the sake of example only, without limiting the scope of the invention. The reference figures quoted below refer to the attached drawings.

### Brief description of the drawings

FIG. 1 is a schematic representation of a side view of an electrospinning setup according to the prior art.
FIG. 2 is a schematic representation of a perspective view of an electrospinning device in operation according to an embodiment of the present invention.
FIG. 3 is a schematic representation of a perspective view of an electrospinning device in operation according to another embodiment of the present invention.
FIG. 4 is a schematic representation of a perspective view of jacketed tubes for temperature control of the solution or melt for use in embodiments of the present invention.
FIG. 5 is a schematic representation of a planar view of the positioning of the outlets for use in an electrospining device according to embodiments of the present invention.
FIG.6 is a magnified picture of a nanofibrous polymeric structure obtained in a comparative experiment.
FIG.7 is a magnified picture of a nanofibrous polymeric structure according to an embodiment of the present invention.
FIG.8 is a magnified picture of a nanofibrous polymeric structure obtained in a comparative experiment.
FIG.9 is a magnified picture of a nanofibrous polymeric structure according to an embodiment of the present invention.
FIG.10 is a magnified picture of a nanofibrous polymeric structure according to an embodiment of the present invention.
FIG.11 is a magnified picture of a nanofibrous polymeric structure obtained in a comparative experiment.
FIG.12 is a magnified picture of a nanofibrous polymeric structure according to an embodiment of the present invention.
FIG.13 is a magnified picture of a nanofibrous polymeric structure obtained in a comparative experiment.
FIG.14 is a magnified picture of a nanofibrous polymeric structure according to an embodiment of the present invention.
FIG.15 is a magnified picture of a nanofibrous polymeric structure according to an embodiment of the present invention.
FIG.16 is a magnified picture of a nanofibrous polymeric structure according to an embodiment of the present invention.
FIG.17 is a table summarizing advantages of embodiments of the present invention.

### Description of illustrative embodiments

The present invention will be described with respect to particular embodiments and with reference to certain drawings but the invention is not limited thereto but only by the claims. The drawings described are only schematic and are non-limiting. In the drawings, the size of some of the elements may be exaggerated and not drawn on scale for illustrative purposes. The dimensions and the relative dimensions do not correspond to actual reductions to practice of the invention.

Furthermore, the terms first, second, third and the like in the description and in the claims, are used for distinguishing between similar elements and not necessarily for describing a sequence, either temporally, spatially, in ranking or in any other manner. It is to be understood that the terms so used are interchangeable under appropriate circumstances and that the embodiments of the invention described herein are capable of operation in other sequences than described or illustrated herein.

It is to be noticed that the term "comprising", used in the claims, should not be interpreted as being restricted to the means listed thereafter; it does not exclude other elements or steps. It is thus to be interpreted as specifying the presence of the stated features, integers, steps or components as referred to, but does not preclude the presence or addition of one or more other features, integers, steps or components, or groups thereof. Thus, the scope of the expression "a device comprising means A and B" should not be limited to devices consisting only of components A and B. It means that with respect to the present invention, the only relevant components of the device are A and B.

Reference throughout this specification to "one embodiment" or "an embodiment" means that a particular feature, structure or characteristic described in connection with the embodiment is included in at least one embodiment of the present invention. Thus, appearances of the phrases "in one embodiment" or "in an embodiment" in various places throughout this specification are not necessarily all referring to the same embodiment, but may. Furthermore, the particular features, structures or characteristics may be combined in any suitable manner, as would be apparent to one of ordinary skill in the art from this disclosure, in one or more embodiments.

Similarly it should be appreciated that in the description of exemplary embodiments of the invention, various features of the invention are sometimes grouped together in a single embodiment, figure, or description thereof for the purpose of streamlining the disclosure and aiding in the understanding of one or more of the various inventive aspects. This method of disclosure, however, is not to be interpreted as reflecting an intention that the claimed invention requires more features than are expressly recited in each claim. Rather, as the following claims reflect, inventive aspects lie in less than all features of a single foregoing disclosed embodiment. Thus, the claims following the detailed description are hereby expressly incorporated into this detailed description, with each claim standing on its own as a separate embodiment of this invention.

Furthermore, while some embodiments described herein include some but not other features included in other embodiments, combinations of features of different embodiments are meant to be within the scope of the invention, and form different embodiments, as would be understood by those in the art. For example, in the following claims, any of the claimed embodiments can be used in any combination.

In the description provided herein, numerous specific details are set forth. However, it is understood that embodiments of the invention may be practiced without these specific details. In other instances, well-known methods, structures and techniques have not been shown in detail in order not to obscure an understanding of this description.

The invention will now be described by a detailed description of several embodiments of the invention. It is clear that other embodiments of the invention can be configured according to the knowledge of persons skilled in the art without departing from the technical teaching of the invention, the invention being limited only by the terms of the appended claims.

In a first aspect, the present invention relates to an electrospinning device for producing fibrous structures such as e.g. nanofibrous structures. In an embodiment of the first aspect, the electrospinning device comprises two or more outlets, advantageously three or more outlets. The outlets may be of any nature known by the person skilled in the art to be suitable for electrospinning. The outlets are adapted for outputting material, e.g. solution or melt material to be used for the production of the fibers. For instance, the outlets may be nozzles, needles such as e.g. metalic needles, small holes or the likes. The two or more outlets are separated from one another by a distance of at least 1 cm. For instance, the outlets may be separated by a distance of 1 to 100 cm. It has surprisingly been found that by separating the outlets by 1 or more cm, the fibrous structures obtained were stronger, more porous and were comprising straighter fibers than for smaller spacing. The relatively large distance between the outlets (e.g. needles) allows an improved evaporation of the solvent, thus resulting in an improved porosity of the fibrous structure obtained. Without being bound by theory this effect may result from a more complete fiber formation process at the moment of collection of those fibers. Advantageously, the distance between the two or more outlets is at least 4 cm, most advantageously 6cm or more. The maximum spacing is arbitrary and will for instance depend on the porosity one wishes to achieve. For a spacing of 1 cm or above between the outlets, the fibers constituting the fibrous structure acquire a surprising straightness over distances of 5 µm or more, 10 µm or more or even 20 µm or more as can be seen e.g. in Fig. 7. In parallel or in addition to this surprising straightness, a majority of the fibres (i.e. 50% or more) constituting the fibrous structure becomes cross-link free, i.e. not cross-linked to neighboring fibers. The majority of the fibres is e.g. substantially cross-link free with respect to neighboring fibers at their contact points. According to embodiments of the present invention, devices are obtained that provide fibres that are cross-link free and thus not linked to each other, i.e. wherein the majority of the fibres, e.g at least 50%, advantageously at least 70%, more advantageously at least 90%, even more advantageously 95% remains independent. Cross link free thereby may be less than 1 cross link per 1 mm fiber length, advantageously less than 1 cross link per 5 mm fiber length, more advantageously less than 1 cross link per 1 cm fiber length, still more advantageously less than 1 cross link per 5 cm fiber length, even more advantageously without cross links over the full length of the fibre. This effect is particularly pronounced for outlets separated by 4 cm or more. When three or more outlets are used, the outlets (e.g. needles) are advantageously arranged in sets of triangles with a distance between each outlet (e.g. needle) of minimum 1 cm and maximum 100 cm, more advantageously of minimum 4cm and maximum 100cm. The total number of outlets is not limited to a maximal value. For instance, the total number of outlets used in a configuration may be between 2 and 20000. Advantageously, the total number of outlets, e.g. needles, used in a configuration is between 3 (see FIG. 5A) and 500 (see FIG. 5B). Different rows, such as e.g. neighbouring rows, of outlets may be parallel but shifted with respect to the corresponding position of the outlets with respect to each other. The latter may be evaluated with respect to the average direction of the relative movement of the second planar surface. The configuration of the outlets may be such that the outlets are positioned in triangular shaped groups of outlets. The set of two or more outlets is positioned in a first plane, i.e. in a surface which is not curved and not circular but has a planar shape. In other words, the different outlets have their output opening in the same plane. The surface defined by the plane is not necessarily solid or substantial, i.e. not necessarily comprised in a solid surface. In some embodiments, the first plane exist solely as a geometrical concept and the outlets are held in the first plane by e.g. a frame or any other structure capable of holding two or more outlets in a plane. In other embodiments, the surface and corresponding plane is material and forms a solid surface comprising the outlets.

The electrospinning device according to the present invention comprises also a second planar surface. The second planar surface is substantially parallel to the first plane and is facing the first plane. The second plane is a surface such as but not limited to a plate (e.g. a metallic plate), a foil or textile structure. The second planar surface may optionally be coated with a perforated or non-perforated layer, e.g. a perforated or non-perforated polymer/plastic layer. The second planar surface may be a planar part of a larger surface not necessarily planar in all its parts. The surface may contain a liquid surface on which the fibers are deposited. The second planar surface advantageously is parallel with the first plane. For instance, the second planar surface may be part of a larger belt comprising winded parts. The second planar surface is adapted for receiving output from the two or more outlets. The ensemble of the first plane and the second planar surface may take any spatial orientation. For instance, this ensemble may be horizontal with the first plane above the second planar surface or with the second planar surface above the first plane. In those cases, the outlets would therefore be oriented downward or upward respectively. For instance the outlets (e.g. needles) are positioned in a lower plate and solution or melt (e.g. polymer solution or melt) jets move upwards the device. In other embodiments, the ensemble of the first plane and the second planar surface is oriented vertically. Other orientations for the ensemble are of course possible (e.g. at 45° or any other angle with the horizon). The ensemble of, on one hand, the first plane comprising the outlets and on another hand the second planar surface is also referred to as a spinneret. At least one of the second planar surface and the set of outlets is adapted to be moveable, i.e. a relative movement may be provided between the second planar surface and the set of outlets. The direction in which the set of outlets may be adapted to move can be either in the first plane or out of the first plane (e.g. perpendicularly to said first plane). The movement of the outlets can also be a combination of a movement in the first plane and out of the first plane. The movement of the outlets is advantageously a reciprocal movement, e.g. a movement between two fixed points. The movement of the second planar surface may be parallel to said second planar surface, orthogonal to said second planar surface or a combination of both. Advantageously, the second planar surface can move continuously in one direction parallel to said second planar surface. Advantageously, the device is adapted for providing a relative movement to the set of outlets and the second planar surface, the relative movement being e.g. a combination of a relative movement in a first direction in the first plane and in a second direction parallel to the first plane and to the second planar surface but different from said first direction. For instance, the second planar surface can be adapted to undergo a relative movement at an angle to the first direction such as optionally substantially perpendicular to said first direction. Said first and second direction can be perpendicular to each other and parallel to said first plane and said second planar surface. In other embodiments, the first and second directions are perpendicular to each other and said first direction is perpendicular to said first plane and said second planar surface. Advantageously, the set of outlets and the second planar surface can move relatively to each other so that the set of outlets moves in one direction in the first plane (e.g. the x-direction), e.g. reciprocally such as e.g. between two inversion points, and the second planar surface moves continuously in a direction perpendicular to the first direction (e.g. the y-direction) but in the plane of said second planar surface. This type of reciprocal movement of the outlets is advantageous because it allows overlapping the output of the outlets as received on the second planar surface from the different outlets. The output of an outlet as received on the second planar surface may be referred to as the fibre umbrellas on the second planar surface. The fibre umbrellas have a high tendency to reject each other due to their charge and can never overlap if the configuration is used as a stationary system, i.e. if there is not at least a reciprocal relative movement between the second planar surface and the set of outlets. The amount of relative reciprocal movement may be selected such that the output of neighbouring outlets at least overlaps. Additionally, the width of the obtained fibrous structure can be increased in this way, i.e. by using a reciprocal movement. Further continuous relative movement between the outlets and the second planar surface allows continuous production of larger fibrous structure surface areas. The relative reciprocal movement between the set of outlets is advantageously subject to a relative movement with respect to the second planar surface with an average speed between 0.1 cm s⁻¹ and 100 cm s⁻¹. The second planar surface is advantageously moveable with a speed between 10 cm h⁻¹ and 100 m h⁻¹. In some embodiments, the distance between the set of outlets and the second planar surface can be varied. For instance, the first set of outlets may move perpendicularly (e.g. in the z direction) to said second planar surface. This enables to implement a fluctuation of the average fiber diameter as a function of thickness of the obtained fibrous structure. Similarly, the second planar surface may move perpendicularly (e.g. in the z direction) to said first plane. Only in those embodiments, i.e. when the distance between the set of outlets and the second planar surface can be varied, the number of outlets can be one or more instead of two or more

The electrospinning device of the present invention further comprises movement means for moving said set of outlets and/or said second planar surface, such as but not limited to one or more motors and one or more actuation means, such as e.g. transmission axis. The movement means may be adapted for inducing one or more of the relative movements as described above.

The electrospinning device of the present invention further comprises a voltage source adapted to apply a potential difference between the outlets and the second planar surface. The voltage source may be a DC-high voltage source able to apply a potential difference selected in the range between 100 and 200000 V over the spinneret, i.e. between the outlets and the second planar surface. For instance, the outlets (e.g. needles) may be electrically in contact with each other through a conductive (e.g. metallic) plate or holding structure. In other embodiments, a semi or non-conductive first material plane (e.g. a plate) or holding structure can be used in combination with means such as e.g. a metallic wire for electrically connecting all the outlets (e.g. needles). The voltage source may be connected to the first plane if this plane is substantive and electroconductive or to means (e.g. wire) for electrically connecting all the outlets (e.g. needles). The second planar surface is advantageously grounded. Optionally it can be used ungrounded (floating) but adapted security measures are then preferably taken.

The electrospinning device of embodiments of the present invention further may comprise at least one recipient for containing a solution or melt to be electrospun from said outlets. The recipient may contain a polymer solution or melt. Alternatively, the receipients may be external to the electrospinning device.

The electrospinning device of embodiments of the present invention advantageously further comprises means for providing the solution or melt to the outlets. The means for providing the solution or melt to the outlets can be any means known by the person skilled in the art. Examples of means for providing the solution or melt to the outlets comprise but are not limited to pumps or syringes among others as well as transfer means such as e.g. tubes.

For instance, each outlet (e.g. needle) can be fed with a solution or melt (e.g. a polymer solution or melt) by an individual means (such as e.g. an individual peristaltic pump). In some embodiments, a multichannel means (such as e.g. a peristaltic pump) can be used in which each channel feeds one individual outlet (e.g. needle). Also a multiple of multichannel means (e.g. pumps) can be used, dependent on the amount of outlets (e.g. needles) that need to be fed with polymer solution or melt. In other embodiments, an anesthesia type pump can be used to feed the outlets (e.g. needles) through syringes filled with polymer solution or melt and positioned in the anesthesia pump. In some embodiments, a multiple amount of outlets (e.g. needles) can be fed by one source being a peristaltic or anesthesia pump. The injection rate (e.g. the pump rate) of solution, e.g. polymer solution, or melt per outlet (e.g. needle) may be between 0.01 and 500 mL h⁻¹.

Solutions or melts usable within the present invention are any solution or melt known by the person skilled in the art to be suitable for forming fibers by electrospinning. The solution or melt can be obtained from polymers. Suitable polymers comprise but are not limited to polyamides, polystyrenes, polycaprolactones, polyacrylonitriles, polyethylene oxides, polylactic acids, polyacrylic acids, polyesteramides, polyvinyl alcohols, polyimides, polyurethanes, polyvinylpyrrolidon, collagen, cellulose and related products, chitosan, methacrylates, silk and combination thereof. The solution or melt may also contain metalic particles so that metal containing fibers can be formed.

As an optional feature, the solutions or melts may contain an additional compound, such as compounds with antibacterial, farmaceutical, hydrophobic/hydrophilic, anti corrosion, catalytic, oxidative/reductive and other properties.

The electrospinning device of the present invention may optionally further comprise a surrounding element, i.e. an element surrounding the other elements of the electrospinning device. For instance, the surrounding element can form a jacket around the spinneret and prevents the spinneret from instability such as air turbulence and/or allow solvent recuperation. Air turbulence are advantageously avoided in the spinneret because it may cause instability in the melt or solution jets and the fibre umbrellas produced by those jets on the second planar surface. The surrounding element may for instance be composed of plates of a non-conductive material connected to each other to form a closed embodiment, i.e. an enclosure.

The electrospinning device of the present invention may further comprise one or more optional temperature control means/systems. Those temperature control means may be added to the electrospinning device for instance in order to obtain higher reproducibility in fibre production. Fluctuations of temperature can have its influence on the evaporation rate of the solvent and thus on the final dimensions of the fibres and the porosity of the structures. Temperature controlling means are therefore advantageous. The solution or melt in the recipient may be temperature conditioned by using containers for (e.g. a liquid bath such as an oil or water bath) temperature control. The control of the temperature can also be operated during the solution transport from the recipient to the outlets via jacketed tubes that are connected directly or indirectly with a cooling/heating system such as said containers for temperature control. The spinneret may be temperature controlled by using means for bringing heated/cooled air in the spinneret. For instance, the electrospinning device of the present invention may comprises a temperature control system that allows to control the temperature in the range 280-1500 K.

In Fig. 2, an electrospinning device according to one particular embodiment of the present invention is presented together with geometrical axes x, y and z. The z axis is the vertical axis while the x and the y axis defines two horizontal axis perpendicular to each other. This device comprises a high voltage source 9, a spinneret, said spinneret comprising a number of outlets 11 such as e.g. needles which are positioned in a first plane, e.g. comprised in a first planar plate 12, and a second planar surface 13. The system also comprises means 10 for providing a solution or melt to the outlets and means 21 for providing a relative movement of the set of outlets 11 with respect to the second planar surface 13. The device may comprise a recipient 20 and a transfer means 22 for providing solution or melt to the outlets.

In operation, the device depicted in Fig.2 operates as follow: A voltage is set between the outlets 11 and the second planar surface 13. A liquid or melt to be electrospun is transferred from the recipient 20 to the outlets 11 via the transfer means 22 by the action of means 10 for providing a solution or melt to the outlets. The relative movement can be obtained by moving the outlets, e.g. by moving the first planar plate, reciprocally in the X direction by the operation of movement means 21 for moving the set of outlets. Simultaneously, the second planar surface may be moved continuously in the Y direction while collecting the fibrous structure formed by the overlap of the umbrellas caused by the melt or solution jets 19.

In Fig. 3, an electrospinning device according to another particular embodiment of the present invention is presented. It comprises all elements present in Fig. 2, and further comprises a means 18 for bringing heated/cooled air in the spinneret, a container for temperature control 17, and a surrounding element 14.

In Fig. 4, shows jacketed tubes comprising an inner tube 16 for solution or melt transport and a jacket 15 for liquid (e.g. oil) based temperature control.

According to the present aspect, the device furthermore may be adapted for generating a laminated fibrous structure, by altering the distance between the outlets and the second planar surface in a controlled way. The device therefore may comprise a controller for controlling movement of the outlets and the second planar surface during the production process of the fibrous structure. The controller may be adapted for selecting a first distance between the outlets and the second planar surface for obtaining a first layer of fibres and selecting one or more other distances between the outlets and the second planar structure for obtaining one or more further layers of fibres with different properties.

In a second aspect, the present invention relates to a method for producing fibrous structures. This method comprises the steps of applying a potential difference, i.e. a voltage between a set of two or more outlets and a second planar surface, moving said set of outlets and said second planar surface relatively to each other, and providing a solution or melt to the outlets. wherein the outlets are separated from one another by a distance of at least 1 cm, The method may advantageously be performed with a system as described in the first aspect. The potential difference may be selected in the range between 100 and 200000 V. The movement step may be performed by actuating means for moving said set of outlets and/or said second planar surface. As a result, at least one of the second planar surface and the set of outlets is moved. The direction in which the set of outlets may move can be either in the first plane or out of the first plane (e.g. perpendicularly to said first plane). The movement of the outlets can also be a combination of a movement in the first plane and out of the first plane. The movement of the outlets may be a reciprocal movement, e.g. a movement between two fixed points. The movement of the second planar surface may be parallel to said second planar surface, orthogonal to said second planar surface or a combination of both. Advantageously, the second planar surface is moved continuously in one direction parallel to said second planar surface. Advantageously, the set of outlets is moved in a first direction in the first plan and the second planar surface is moved in a second direction parallel to the first plan and to the second planar surface but different from said first direction. For instance, the second planar surface can be moved at an angle to the first direction such as optionally substantially perpendicular to said first direction. Said first and second direction may be perpendicular to each other and parallel to said first plane and said second planar surface. Advantageously, the set of outlets and the second planar surface are moved relatively to each other so that the set of outlets moves in one direction in the first plane (e.g. the x-direction) between two inversion points and the second planar surface moves continuously in a direction perpendicular to the first direction (e.g. the y-direction) but in the plane of said second planar surface. The set of outlets may move with an average speed between 0.1 cm S⁻¹ and 100 cm S⁻¹. The second planar surface may move with a speed between 10 cm h⁻¹ and 100 m h⁻¹.

The solution or melt may be kept in a recipient which may but does not have to be temperature controlled. Providing the solution or melt can be performed by solution or melt actuating means for providing the solution or melt to the outlets. Those means such as e.g. a pump transfer the solution or melt to the outlets via transfer means which may but do not have to be temperature controlled. Once at an outlets, the solution or melt forms a droplet from which a filament will be drawn and projected toward the second planar surface under the action of the potential difference. The second planar surface acts therefore as a collecting surface. The shape of the jet of solution or melt leaving an outlet is usually conical and forms a so-called umbrella, i.e. a covered area on the second planar surface. Due to the relative movement of the outlets toward the second planar surface, the umbrella overlaps and form a fibrous structure such as a mat composed of fibres. The fibrous structures can in a later stage be recovered from the second planar surface by any method well known to the person skilled in the art.

In embodiments of the second aspect, the present invention also relates to a method for producing fibrous structures having a porosity of at least 65%, said method comprising the steps of applying a potential difference between a first surface and a second surface, said first surface comprising three or more outlets, providing a relative movement between said first surface and said second surface resulting in movement of the first surface in a first direction while simultaneously moving said second surface in a second direction substantially perpendicular to said first direction, and providing a solution or melt to said outlets, wherein the three or more outlets are separated from one another by a distance of at least 1 cm.

In a third aspect, the present invention relates to a fibrous structure comprising a majority, i.e. 50% or more of straight fibers. In one embodiment, the fibrous structure forms a mat. The method of the second aspect applied to the device of the first aspect permits to obtain fibrous structures having outstanding properties. A remarkable property being the straightness of the fibers comprised in the obtained fibrous structure. This straightness can be readily and directly observe in magnified pictures of the fibrous structures. This can for instance be observed in Fig. 7, 9, 10, 12, 14, 15 and 16. An image analysis permits to determine that the majority of the fibers (i.e. 50% or more) comprised in the fibrous structure are straight, i.e. consists of a majority of segments (i.e. 50% or more) substantially straight over a distance of 5 µm. By substantially straight, it must be understood that the major axis of the fibre, i.e. along the direction of the fibre, changes over an angle less than 45°, e.g. less than 30°, or e.g. less than 15° or e.g. less than 5°, considering a distance of 10micrometer over which the angle change was measured. This angle is the largest angle which can be measured between tangents at two points of the major axis over the length of the fiber considered. The standard deviation to linearity over the distance in question may be not exceeding 5%.

The present invention also relates to a fibrous structure, e.g. microfibrous or nanofibrous structure wherein surprisingly a majority of the fibers (i.e. 50% or more) comprised are substantially cross-link free. The fibrous structure is an electrospun fibrous structure, it is a structure made by electrospinning. They are advantageously not cross-linked to neighboring fibers. Cross-linking thereby means that a link occurs between two fibres, not just that two fibers are touching. This is the result of the spacing between the outlets being at least 1 cm. Without being bound by theory, it is believed that this effect is due to an easier and therefore faster evaporation evaporation of the solvent during during the fibres formation. It is believed that for spacing between the outlets inferior to 1 cm, the solvent takes too much time to evaporate during the fibres formation. This leads to fusing of adjacent fibres and therefore to crosslinks. If the fibrous structure is made from a melt, the problem may be an incomplete elimination of the heating effect occurring when outlets are too close to each other. The fiber formation then is not complete and a sort of intermediate phase between melt and solid then may be present, allowing formation of cross-linked fibres. This effect is for instance clearly visible in Fig.6, 8, 11 and 13. Another remarkable feature of the fibrous structures obtained is that they have a porosity of at least 65%, advantageously between 65 and 99%.

The present invention also relates to a fibrous structure wherein the thickness of the fibres is uniform, i.e. the standard deviation of the thickness throughout the fibrous structure does not exceed 80%, advantageously 50%, most advantageously 20%

The present invention also relates to a fibrous structure comprising more or all of the above identified properties. As an optional feature, the fibrous structures according to the present invention can be made comprising a majority of fibers (i.e. 50% or more) randomly oriented, i.e. not oriented in a particular direction (e.g. not alligned). The last effect is helpful in achieving an increased porosity. In embodiments where the second planar surface moves continuously in one direction, this effect can be obtained for example by choosing a speed for the second planar surface between 10 cm h⁻¹ and 100 m h⁻¹. As an optional feature, the diameter of a majority of the fibres (i.e. 50% or more of the fibers) comprised in the fibrous structures of the present invention have a diameter of 3 nm or higher, advantageously 10 nm or higher. As an optional feature, the diameter of a majority of the fibres (i.e. 50% or more) comprised in the fibrous structures of the present invention have a diameter of 2000 nm or lower, advantageously 800 nm or lower, most advantageously 700 nm or lower. When the fibers have an average diameter of 800 nm or lower, they will be referred to as nanofibers and the fibrous structures made therefrom as nanofibrous structures. As an optional feature, the diameter of a majority of the fibers (i.e. 50% or more) comprised in the fibrous structures of the present invention have a diameter of 3 to 2000 nm, advantageously between 10 and 2000 nm, advantageously between 3 and 800 nm, more advantageously a diameter of 10 to 700 nm. As another optional feature, the fibrous structures obtained have a width between 15 and 10000cm.

In embodiments of the third aspect of the present invention, the fibrous polymeric structures have a porosity of at least 65% and a width comprised between 15 and 10000 cm.

In some embodiments of the third aspect, the fibrous structures are obtained laminated, i.e. multi-layered. Advantageously, the average fibre diameter is different for each pair of adjacent layers within the fibrous structure. This may be achieved by using a different distance between the set of outlets and the second planar surface for each layer. The obtained laminated fibrous structures have a number of advantages compared to their non-laminated counter parts. Firstly, the combination of layers with small fiber diameter and layers with somewhat bigger fibers improve on the overall strength of the fibrous structure. Secondly, the absorption/release properties of the fibrous structure can be optimized as a function of application and this in a single production step and finally, multitasking and multifunctionality can be obtained by using a laminated structure, such as multilevel filtration in one single multilayered structure.

In Fig. 17, different ways are described to obtain laminated structures with minimum 2 layers. In column three is a visualization of the movement of the set of outlets to obtain the desired laminated structure (see Fig. 17).

In a first specific embodiment (Fig. 17, nr. 1), a fibrous structure with two layers 23 and 24 is obtained, each layer being comprised of fibres of different diameter. To obtain such a fibrous structure, first the set of outlets moves in y-direction from left to right and back with a preset frequency while the second planar surface is optionally moved continuously in the x-direction. After that the desired thickness of the first layer is obtained, the distance between the set of outlets and the second planar surface is adapted (e.g. reduced). That can be performed e.g. by moving from left to right (opposite is also possible) the set of outlets, while simultaneously moving the set of outlets downward in the z-direction. When it has reached its destination the plate continues to move from left to right in the lower position, resulting in the formation of a second layer with different diameters of the fibers. In a second specific embodiment (Fig 17, nr. 2), which is similar to the first one, except that the two layers are inverted in relative position, the set of outlets moves from a lower to a higher position (instead of starting at the higher and moving to the lower) after that the first layer of fibers is formed. In a third specific embodiment (Fig 17, nr. 3) a three layer structure is obtained by moving the set of outlets from left to right and back with a preset frequency, then going down to its second position where it continues to move between two points in y-direction. Finally, the set of outlets returns upward to its initial position and finishes the procedure again with a preset number of times moving between 2 points in the upper position. In yet another specific embodiment (Fig 17, nr. 4) the set of outlets starts in its lower position, after formation of the first layer it moves to its upper position and finally returns to its initial lower position to produce the third layer. A high number of other embodiments is possible, e.g. with more than three layers, and by stacking layers of fibers, having more than two different average diameters of the individual fibers. These embodiments can be obtained by switching many times the position of the outlets in the z-direction and by using more than two positions at which the upper plate stays for formation of an individual layer of the fibrous structure.

### EXAMPLE 1

Polyethylene oxide (PEO) with molecular weight of 300.000 g mol⁻¹ is dissolved in water to obtain a solution of 12% PEO. The solution is pumped to a set of needles with a multitude of multichannel peristaltic pumps, with a flow rate of 10 mL h⁻¹ per needle. In the spinneret an electrical field of about 800 V cm⁻¹ is applied over the upper and lower element in order to allow electrospinning of the polymer solution. Temperature control was performed at 298 K. In one setup 3 needles were used which were positioned at a distance of 2 mm (FIG. 6); in another setup the needles were positioned 6 cm from each other (FIG. 7). In the first setup the nanofibrous structures are less clear and have reduced porosity. With 3 needles a nanofibrous structure production rate of about 0.4 m h⁻¹ was obtained over a width of 60 cm, having a uniform thickness of 0.44±0.02 mm.

### EXAMPLE 2

Polyester amide (PEA) with molecular weight of about 20.000 g mol⁻¹ is dissolved in chloroform to obtain a solution of 25% PEA. The solution is pumped to a set of needles with a multitude of multichannel peristaltic pumps, with a flow rate of 15 mL h⁻¹ per needle. In the spinneret an electrical field of about 1000 V cm⁻¹ is applied over the upper and lower element in order to allow electrospinning of the polymer solution. Temperature control was performed at 298 K. In one setup 3 needles were used which were positioned at a distance of 2 mm (FIG. 8); in another setup the needles were positioned 6 cm from each other (FIG. 9). With 3 needles a nanofibrous structure production rate of about 0.5 m h⁻¹ was obtained over a width of 60 cm, having a uniform thickness of 0.50±0.02 mm.

### EXAMPLE 3

Cellulose acetate (CA) with molecular weight of 30.000 g mol⁻¹ is dissolved in cyclohexanol to obtain a solution of 8% CA. The solution is pumped to a set of needles with a multitude of multichannel peristaltic pumps, with a flow rate of 10 mL h⁻¹ per needle. In the spinneret an electrical field of about 1100 V cm⁻¹ is applied over the upper and lower element in order to allow electrospinning of the polymer solution. Temperature control was performed at 298 K. In one setup 3 needles were used which were positioned at a distance of 2 mm; in another setup the needles were positioned 6 cm from each other (Fig. 10). For the first setup no nanofibrous structure was obtained. With 3 needles a nanofibrous structure production rate of about 0.3 m h⁻¹ was obtained over a width of 60 cm, having a uniform thickness of 0.40±0.02 mm.

### EXAMPLE 4

CA with molecular weight of 30.000 is dissolved in Aceton/EtOH to obtain a solution of 12% CA. The solution is pumped to a set of needles with a multitude of multichannel peristaltic pumps, with a flow rate of 6 mL h⁻¹ per needle. In the spinneret an electrical field of about 700 V cm⁻¹ is applied over the upper and lower element in order to allow electrospinning of the polymer solution. Temperature control was performed at 298 K. In one setup 3 needles were used which were positioned at a distance of 2 mm (Fig. 11); in another setup the needles were positioned 6 cm from each other (FIG. 12). With 3 needles a nanofibrous structure production rate of about 0.3 m h⁻¹ was obtained over a width of 60 cm, having a uniform thickness of 0.40±0.02 mm.

### EXAMPLE 5

CA with molecular weight of 40.000 is dissolved in Aceton/DMA to obtain a solution of 12% CA. The solution is pumped to a set of needles with a multitude of multichannel peristaltic pumps, with a flow rate of 10 mL h⁻¹ per needle. In the spinneret an electrical field of about 800 V cm⁻¹ is applied over the upper and lower element in order to allow electrospinning of the polymer solution. Temperature control was performed at 298 K. In one setup 3 needles were used which were positioned at a distance of 2 mm (FIG. 13); in another setup the needles were positioned 6 cm from each other (FIG. 14). With 3 needles a nanofibrous structure production rate of about 0.18 m h⁻¹ was obtained over a width of 60 cm, having a uniform thickness of 0.30±0.02 mm.

### EXAMPLE 6

Polyamide 6/6 (PA66) is dissolved in formic acid to obtain a solution of 14% PA66. The solution is pumped to a set of needles with a multitude of multichannel peristaltic pumps, with a flow rate of 5 mL h⁻¹ per needle. In the spinneret an electrical field of about 4800 V cm⁻¹ is applied over the upper and lower element in order to allow electrospinning of the polymer solution. Temperature control was performed at 298 K. In one setup 3 needles were used which were positioned at a distance of 2 mm; in another setup the needles were positioned 6 cm from each other (FIG. 15). In the first setup a solid structures instead of nanofibrous structure was obtained. With 3 needles a nanofibrous structure production rate of about 0.3 m h⁻¹ was obtained over a width of 60 cm, having a uniform thickness of 0.40±0.02 mm.

### EXAMPLE 7

Chitosan with molecular weight of about 250.000 g mol⁻¹ is dissolved in acetic acid (90%) to obtain a solution of 3% Chitosan. The solution is pumped to a set of needles with a multitude of multichannel peristaltic pumps, with a speed of 0.5 mL h⁻¹ per needle. In the spinneret an electrical field of about 2000 V cm⁻¹ is applied over the upper and lower element in order to allow electrospinning of the polymer solution. Temperature control was performed at 298 K. In one setup 3 needles were used which were positioned at a distance of 2 mm; in another setup the needles were positioned 6 cm from each other (Fig. 16). For the first setup no nanofibrous structure was obtained. With 3 needles a nanofibrous structure production rate of about 0.01 m h⁻¹ was obtained over a width of 60 cm, having a uniform thickness of 0.30±0.02 mm.

### EXAMPLE 8

TiO₂ nanofibrous structures were obtained from dissolving Ti-isopropoxide and polyvinylpyrrolidon with molecular weight of 900.000 g mol⁻¹ in EtOH to obtain a solution. The solution is pumped to a set of needles with a multitude of multichannel peristaltic pumps, with a speed of 16 mL h⁻¹ per needle. In the spinneret an electrical field of about 1800 V cm⁻¹ is applied over the upper and lower element in order to allow electrospinning of the polymer solution. Temperature control was performed at 298 K. In one setup 3 needles were used which were positioned at a distance of 2 mm; in another setup the needles were positioned 6 cm from each other. With 3 needles a nanofibrous structure production rate of about 0.1 m h⁻¹ was obtained over a width of 60 cm, having a uniform thickness of 0.40±0.02 mm.

### EXAMPLE 9

PA66 is dissolved in formic acid/acetic acid to obtain a solution of 15% PA66. The solution is pumped to a set of needles with a multitude of multichannel peristaltic pumps, with a speed of 6 mL h⁻¹ per needle. In the spinneret an electrical field of about 5000 V cm⁻¹ is applied over the upper and lower element in order to allow electrospinning of the polymer solution. Temperature control was performed at 298 K. In one setup 3 needles were used which were positioned at a distance of 2 mm; in another setup the needles were positioned 6 cm from each other. Similar pictures were obtained as in example 6. With 3 needles a nanofibrous structure production rate of about 0.3 m h⁻¹ was obtained over a width of 60 cm, having a uniform thickness of 0.44±0.02 mm.

It is to be understood that although preferred embodiments, specific constructions and configurations, as well as materials, have been discussed herein for devices according to the present invention, various changes or modifications in form and detail may be made without departing from the scope and spirit of this invention. For example, any formulas given above are merely representative of procedures that may be used. Functionality may be added or deleted from the block diagrams and operations may be interchanged among functional blocks. Steps may be added or deleted to methods described within the scope of the present invention. Whereas the present invention has been described with respect to a method for manufacturing, an electrospinning device and the resulting fibrous structures, the present invention also relates to a controller for controlling a relative distance between the outlets and the second planar surface for generating different properties between different layers in a fibrous structure.

## Claims

1. An electrospinning device for producing fibrous structures, said electrospinning device comprising:
- a set of two or more outlets (11) for outputting solution or melt, said two or more outlets being arranged in a first plane (12),
- a second planar surface (13) arranged parallel to said first plane (12), the second planar surface (13) for receiving output from said two or more outlets (11), wherein said set of two or more outlets (11) and said second planar surface (13) are adapted to move relatively to each other,
- a voltage source (9) for generating a potential difference between said set of two or more outlets (11) and said second surface (13),
- providing means (10) for providing said solution or melt to said outlets,
**characterized in that** at least two neighbouring outlets of said two or more outlets (11) are separated from one another by a distance of at least 1 cm.

2. The device according to claim 1, wherein at least two neigbouring outlets of said two or more outlets (11) are separated from one another by a distance of at least 4 cm.

3. The device according to claim 1, wherein the distance between said two or more outlets (11) is adapted for obtaining a fibrous structure comprising at least 50% of fibers substantially free of cross-links to neighboring fibers.

4. The device according to claim 1 or claim 3, wherein the distance between said two or more outlets (11) is adapted for obtaining a fibrous structure comprising at least 50% of straight fibers.

5. The device according to any of claims 1 to 3, wherein a relative movement between said two or more outlets (11) and said second surface (13) can be applied in a first direction and in a second direction, different from said first direction.

6. The device according to claim 5, wherein said second direction is perpendicular to said first direction.

7. The device according to claim 6, wherein said second direction is parallel to said first plane (12).

8. The device according to claim 6, wherein said second direction is perpendicular to said first plane (12).

9. The device according to any of claims 5 to 8, wherein said two or more outlets (11) are adapted to be movable reciprocally in said first direction.

10. The device according to any of claims 1 to 9, wherein said device comprises control means for varying the diameter of the produced fibres.

11. The device according to claim 10, wherein said means for varying the diameter of the produced fibres are control means for altering the distance between said first plane (12) and said second planar surface (13) during the production of the fibrous structure.

12. An electrospinning device for producing a fibrous structure, said electrospinning device comprising:
- one or more outlets (11) for outputting solution or melt, said two or more outlets being arranged in a first plane (12),
- a second planar surface (13), for receiving output of said two or more outlets, the second planar surface arranged parallel to said first plane (12),
- a voltage source (9) for generating a potential difference between said one or more outlets (11) and said second planar surface (13),
- providing means (10) for providing a solution or melt to said outlets (11),
**characterized in that** said device comprises control means for varying the diameter of the produced fibres.

13. The electrospinning device according to claim 12, wherein said means for varying the diameter of the produced fibres are control means for altering the distance between said first plane (12) and said second planar surface (13) during the production of the fibrous structure.

14. A method for producing fibrous structures, said method comprising the steps of:
(i) moving a set of two or more outlets (11), for outputting solution or melt, said set being comprised in a first plane (12), and a second planar surface (13), for receiving output of said two or more outlets, (11) relatively to one another,
(ii) applying a potential difference between said set of two or more outlets (11), and said second planar surface (13), and
(iii) during said moving and applying, providing a solution or melt to said outlets (11),
wherein at least two neighbouring outlets of said two or more outlets (11) are separated from one another by a distance of at least 1 cm.

15. A method according to claim 14 wherein step (i) comprises adapting the distance between said set of two or more outlets (11) and said second planar surface (12).

16. A method for producing fibrous structures, said method comprising the steps of:
(i) adapting the distance between a set of one or more outlets (11) for outputting solution or melt, said set being comprised in a first plane (12), and a second planar surface (13) for receiving output of said two or more outlets,
(ii) applying a potential difference between:
- said set of one or more outlets (11), and
- the second planar surface (13), and
(iii) providing a solution or melt to said outlets (11).

17. The method of claim 16 comprising the steps of:
a) performing step (i) such as to achieve a predefined distance between said set of outlets (11) and said second planar surface (13),
b) while performing step (ii) and step (iii), moving reciprocally at least one of said set of outlets (11) and/or said second planar surface (13) in a first direction and in a second direction perpendicular to the first direction and parallel to said first plane (12),
c) iterating step (a) and step (b) a predetermined number of times,
wherein said the sense of movement is reversed between each iteration.

18. The method for producing fibrous structures according to any of claims 15 to 17, wherein said distance is adapted by providing a relative movement between said set of outlets (11) and said second planar surface (13) in a first direction and a second direction perpendicular to said first direction and perpendicular to said first plane (12).

19. An electrospun fibrous structure, the structure comprising at least 50% of straight fibers, wherein at least 50% of straight fibers consists of 50% or more fibres having segments substantially straight over a distance of 5 µm.

20. An electrospun fibrous structure according to claim 19, comprising at least 50% of fibers that is substantially cross-link free with respect to neighboring fibers.

21. An electrospun fibrous structure according to claim 19 or claim 20, comprising at least 50% of randomly oriented fibers.

22. An electrospun fibrous structure according to any of claims 19 to 21 having a porosity of at least 65%.

23. An electrospun fibrous structure according to any of claims 19 to 22 wherein 50% or more of its fibers having an average diameter between 3 and 2000 nm.

24. An electrospun fibrous structure according to any of claims 19 to 23, said fibrous structure comprising two or more adjacent layers, wherein each of said layers is composed of fibers having an average diameter different from the average diameter of the fibers of an adjacent layer.

25. An electrospun fibrous structure comprising two or more adjacent layers, wherein each of said layers is composed of fibers having an average diameter different from the average diameter of the fibers of an adjacent layer.

26. A filtrating or an absorbing device comprising an electrospun fibrous structure according to any of claims 19 to 25.

27. A controller for controlling an electrospinning device for performing a method according to any of claims 14 to 18.
